# EUROPEAN PATENT SPECIFICATION

(11) **EP 1 545 841 B1**
(45) Date of publication and mention of the grant of the patent: **08.12.2010**
(21) Application number: 03759604.6
(22) Date of filing: 01.10.2003
(51) Int. Cl.: B26B 21/56, B26B 19/38, B26B 21/58

(54) **ZIRCONIA BASED BLADES AND FOILS FOR RAZORS AND A METHOD FOR PRODUCING SAME**
KLINGEN UND SCHERFOLIEN AUF ZIRKONIUMDIOXIDBASIS FÜR RASIERER UND VERFAHREN ZUR HERSTELLUNG DERSELBEN
LAMES ET FEUILLES A BASE DE ZIRCONE POUR RASOIRS ET PROCEDE DE FABRICATION ASSOCIE

(30) Priority: 01.10.2002 GB 0222712; 10.10.2002 GB 0223567; 15.10.2002 GB 0223882
(43) Date of publication of application: 29.06.2005
(73) Proprietor: EVEREADY BATTERY COMPANY, INC., St. Louis, MO 63141 (US)
(72) Inventor: DENNE, William, Anthony, The Lane House, Cambridge CB2 5EL (GB)
(74) Representative: von Kreisler Selting Werner
(86) International application number: PCT/US2003/030958
(87) International publication number: WO 2004/030875

(56) References cited:
- DE-C- 641 901
- FR-A- 2 584 333
- US-A- 2 989 804
- US-A- 3 870 776
- US-A- 4 105 493
- US-A- 4 483 068
- US-A- 4 552 832
- US-A- 5 018 274
- US-A- 5 604 983
- US-A- 5 750 956
- US-A1- 2003 063 155

## Description

This application claims the priority of British Provisional Application No. 0222712.2 filed on October 1, 2002 entitled "Zirconia Razor Foil"; British Provisional Application No. 0223567.9 filed on October 10, 2002 entitled "Ceramic Razor Blades"; and British Provisional Application No. 0223882.2 filed on October 16, 2002 entitled "Perforated Razor Blade".

### FIELD OF THE INVENTION

This invention relates generally to blades and foils for razors, and more particularly relates to zirconia based blades and foils for razors, as well as methods for producing same.

### BACKGROUND OF THE INVENTION

Electric razors with cutting foils and wet shave razors with cutting blades have been in use for many decades. With respect to electric razors, they comprise a pierced foil and cutter. The foil is generally electroformed from nickel, which provides a very sharp edge but of limited hardness. Electric razor foils are generally made by electroforming nickel. This is a relatively expensive process and the hardness of the resulting nickel cutting edges is not that high.

With respect to wet shave razors, the razor blades traditionally have a straight cutting edge that extends the length of the razor head. Safety razors have guards to control the position of the skin with respect to the cutting edge, so that the cutting edge rides over the skin but cuts protruding hair. Such razor blades have traditionally been made from high quality carbon steel. The innovation of using stainless steel has been fraught with the difficulty of forming and holding an ultra sharp edge. Ground ceramic razor blades tend to have a ragged microstructure rather than rounded, and consequently dig into skin rather than sliding over it.

Accordingly, it is a general object of the present invention to provide zirconia based blades and foils, and methods of fabrication thereof, that overcome the above-identified drawbacks of prior razors.

### SUMMARY OF THE INVENTION

The present invention resides in a method of fabricating a blade for a wet shave razor. A substrate is provided including a combustible surface. A zirconia based ink is generated on the combustible surface such that the ink wets the substrate and edges of the ink slightly to form a plurality of sharply pointed meniscus to serve as cutting surfaces. The ink is fired to burn away the combustible surface and to harden a rounded, sharp edge on the plurality of meniscus. Preferably, the sharp edges of the meniscus have an edge radius of about 50 nanometers or less.

### BRIEF DESCRIPTION OF THE DRAWINGS

FIG. 1A is a top plan view of a razor blade substrate defining an array of rectangular slots serving as cutting edges in accordance with the present invention.
FIG. 1B is a top plan view of a razor blade substrate defining an array of staggered rectangular slots serving as cutting edges in accordance with another embodiment of the present invention.
FIG. 1C is a top plan view of a razor blade substrate defining an array of diamond-shaped slots serving as cutting edges in accordance with a further embodiment of the present invention.
FIG. 2 is an elevational, cross-sectional view of the razor blade of FIG. 1 showing a curved contour of the blade in contact with the skin of a user.

### DETAILED DESCRIPTION OF THE PREFERRED EMBODIMENTS

In accordance with the present invention, an electric razor foil can be made from zirconia ceramic. The zirconia may be partially or fully stabilized. The foil may be fabricated by screen printing the foil plan form onto a hydrophilic surface with a zirconia based ink, such that flow of the ink under surface tension forces generates very sharp edges to the ceramic foil. The planar hydrophilic surface may be combustible so that it vanishes during firing. The surface is preferably a plastic film of good surface finish. The foil network may be biaxially extensible to conform to the skin. The cutter may also be in the form of a zirconia foil. The zirconia print and plastic film may be formed prior to firing. Vacuum forming may be appropriate. Appropriate binders and plasticisers in the zirconia ink may stop cracking of the ceramic print during the forming process.

Partially stabilized zirconia has the hardness and toughness of tool steel. It has excellent wear characteristics and takes a very keen edge. While it is much more expensive, the quantity in a razor foil is minimal and it may be fabricated more cheaply than electroforming.

A razor foil pattern may be precisely screen printed onto a plastic film with a zirconia ink. If the film is slightly hydrophilic it may be arranged, by controlling the ink properties, such that the edges of the print may run slightly under the influence of surface tension forces to provide an extremely sharp edge. Even a low cost plastic film may have a surface finish approaching optical quality and the zirconia print will accurately reproduce this.

The printed plastic film may be fired in the conventional manner. The plastic will burn away at a low temperature and the zirconia will form a very thin foil of extreme toughness. It will maintain its sharpness for a long time.

The foil pattern can be printed in a manner that permits biaxial extension to follow the contours of the skin. A cutter in foil form can also be fabricated which will follow the outer foil and provide a flexible cutting surface.

The printed plastic may be vacuum formed if desired. This permits the forming of the profiled cutters used in current multi head shavers. The form may also be exploited to assist with maintaining dimensional stability during the firing process.

Further in accordance with the present invention, razor blades can be fabricated from a ceramic ink that is screen printed on a combustible surface and then fired. The ceramic is preferably stabilized or partially stabilized zirconia. The combustible surface is preferably a plastic film of high surface finish. The ink vehicle and combustible surface may be so chosen that the ink wets the combustible surface.

Stabilized zirconia forms exceptional cutting blades. It is extremely strong, tough and hard. In thin sheets it may be very pliable. It has been discovered to be an excellent medium for razor blade fabrication. The raw material is very expensive compared with steel and is expensive to diamond machine. Cutting edges in zirconia are conventionally created by diamond machining, but this process produces ragged edges on a micro-scale which tend to dig into skin rather than slide over it. This, of course, is disastrous in a razor blade.

Screen printing of ceramic inks is a well known mass production technique in hybrid electronics. This produces a thin film of very finely controlled thickness at very low cost. The ink comprises very finely powdered ceramic in a binder and solvent. It is possible to choose the composition of ink such that it wets the substrate and the edges of the print flow slightly to form a sharply pointed meniscus. On firing, the substrate may burn away and the meniscus will form a very sharp edge. The firing process causes the finely powdered grains to sinter into a solid mass. This process may be exploited to form an edge to the blade which is rounded on a microscale. With modern milling techniques, the powder particle size may be some tens of nanometers. It is therefore possible to organize the firing to produce a blade with an edge radius of about 50 nanometers or less.

The ceramic will take the surface finish of the substrate on the printed side, which may approach optical quality for many plastic films. If this is the side that faces the skin, a very smooth blade will result. Screen printing produces very thin layers with excellent reproducibility. Zirconia blades as thin as about 0.025 mm are feasible. By using thin blades of minimum width, blade costs of a fraction of a penny are feasible.

This fabrication technique offers the advantages of large scale mass coupled with low materials cost and no finishing processes.

Further in accordance with the present invention, a metallic or ceramic razor blade can be curved and define a plurality of holes or slots, some or all of which incorporate a cutting edge as part or all of their periphery. With reference to FIG. 1A, for example, a razor blade is indicated generally by the reference number 10. The blade 10 defines a plurality of holes or rectangular slots 12 that preferably form an array. As shown in FIG. 1A, the array of slots 12 includes five columns 14, 16, 18, 20 and 22. However, the array can include a fewer or greater number of columns than that illustrated without departing from the scope of the present invention. A portion of the periphery of the slots 12 serve as cutting edges that are well protected within the slots. As a result, the edge of the blade is no longer in need of careful protection.

With respect to the direction of blade movement during a shaving operation as indicated by the arrow A, the longer edges of the rectangular slots 12 are trailing edges 24 and leading edges 26. The blade 10 further defines interconnecting spokes 28 between shorter edges 30 of the rectangular slots 12 for enhancing the rigidity of the blade. A periphery 32 of the blade 10 may be used to retain the blade in a razor.

The leading edges 26 serve as a guard, and the trailing edges 24 serve as the cutting edge. However, the blade 10 can be used in a direction opposite to that indicated by the arrow A. When used in such opposite direction, the edges 24 are the leading edges serving as the guard, and the edges 26 are the trailing edges serving as the cutting edges.

Turning to FIG. 1B, a blade in accordance with another embodiment of the present invention is indicated generally by the reference number 110. Like elements with those shown in FIG. 1A are indicated by like reference numbers preceded by "1". The blade 110 defines a plurality of holes or staggered rectangular slots 112 that form an array. As shown in FIG. 1B, the array of slots 112 includes five columns 114, 116, 118, 120 and 122. The slots in adjacent columns are positioned in staggered relationship to one another to provide a consistent cutting surface along a direction of the blade transverse to that of the direction of movement.

Similar to the previous embodiment, a portion of the periphery of the slots 112 serve as cutting edges. With respect to the direction of blade movement during a shaving operation as indicated by the arrow A, the longer edges of the rectangular slots 112 are trailing edges 124 and leading edges 126. The blade 110 further defines interconnecting spokes 128 between shorter edges 130 of the rectangular slots 112 for enhancing the rigidity of the blade. A periphery 132 of the blade 110 may be used to retain the blade in a razor.

The leading edges 126 serve as a guard, and the trailing edges 124 serve as the cutting edge. However, the blade 110 can be used in a direction opposite to that indicated by the arrow A. When used in such opposite direction, the edges 124 are the leading edges serving as the guard, and the edges 126 are the trailing edges serving as the cutting edges.

Turning to FIG. 1C, a blade in accordance with a further embodiment of the present invention is indicated generally by the reference number 210. Like elements with those shown in the previous embodiments are indicated by like reference numbers preceded by "2". The blade 210 defines a plurality of holes or staggered diamond-shaped slots 212 that form an array. The blade 210 also preferably defines partial or half-diamond-shaped slots 213 at ends of the array for even distribution of cutting surfaces between sides of the blade. As shown in FIG. 1C, the array of slots 212 includes five columns 214, 216, 218,220 and 222. The slots in adjacent columns are positioned in staggered relationship to one another to provide a consistent cutting surface along a direction of the blade transverse to that of the direction of movement.

Similar to the previous embodiments, portions of the periphery of the slots 212 serve as cutting edges. With respect to the direction of blade movement during a shaving operation as indicated by the arrow A, the diamond-shaped slots 212 each include trailing edges 224, 225 and leading edges 226, 227. A periphery 232 of the blade 210 may be used to retain the blade in a razor.

The leading edges 226, 227 serve as a guard, and the trailing edges 224, 225 serve as the cutting edge. However, the blade 210 can be used in a direction opposite to that indicated by the arrow A. When used in such opposite direction, the edges 224, 225 are the leading edges serving as the guard, and the edges 226, 227 are the trailing edges serving as the cutting edges.

With reference to FIG. 2, a blade in accordance with the present invention may have an overall curvature to expose different angles of blade to the skin. A curved blade 310 defines an array of holes or slots 312 in contact with skin 313 of a user during a shaving operation. As shown in FIG. 2, the array of slots 312 includes five columns 314, 316, 318, 320 and 322. With respect to the direction of blade movement during a shaving operation as indicated by the arrow A, a hair 323 is shown being cut by a trailing or cutting edge 324 of one of the holes 312. The curvature and flexibility of the blade 310 may be predetermined to offer the maximum ability to follow skin contours. Several cutting edges 324 may be in contact with the skin simultaneously. The leading edges 326 of the holes or slots 312 control the access of the skin 313 to the cutting edges 324 of the hole 312. The blade may be formed from metal by electroforming or by grinding away dimples in a planar shim. The blade may also be formed by screen printing ceramic ink as an array of holes, and then firing the print. The rheology of the ink may be arranged so that the flow of the periphery of the wet print may form a meniscus which becomes a polished razor edge on firing. The ceramic is preferably partially stabilized or fully stabilized zirconia ceramic. The ceramic may also be ground and polished after firing if desired.

Razor blades traditionally have a straight cutting edge. An array of holes with cutting edges around their periphery in accordance with the present invention provides a longer cutting edge per square millimeter of blade and a tighter control of the angle at which the skin meets the blade. This results in a more rapid and closer shave with less chance of nicking the skin.

In a metal blade, such an array may be made by electroforming. Electroforming is relatively expensive for disposable blades, however, and nickel, which is the only practical metal for this technique, is not exceptionally hard. An alternative is to form an array of indentations in a planar metal shim, and then to grind away the raised bumps to create holes surrounded by a cutting edge.

A better process is to screen print the blade pattern with partially stabilized zirconia ink. If the rheology of the ink and the nature of the substrate are carefully chosen, the edges of the print flow to create a wetting meniscus. On firing, this meniscus naturally creates a polished razor edge.

As will be recognized by those of ordinary skill in the pertinent art, numerous modifications and substitutions may be made to the above-described embodiment of the present invention without departing from the scope of the invention. Accordingly, the preceding portion of this specification is to be taken in an illustrative, as opposed to a limiting sense.

## Claims

1. A method of fabricating a blade for a wet shave razor, comprising the steps of:
providing a substrate including a combustible surface;
generating a zirconia based ink onto the combustible surface such that the ink wets the substrate and the edges of the print flow slightly to form a plurality of sharply pointed menisci to serve as cutting surfaces; and
firing the ink to burn away the combustible surface and to harden a rounded, sharp edge on the plurality of menisci.

2. A method as defined in claim 1, wherein the step of generating includes screen printing the zirconia based ink onto the combustible surface.

3. A method as defined in claim 1, wherein the zirconia based ink includes partially stabilized zirconia.

4. A method as defined in claim 1, wherein the zirconia based ink includes fully stabilized zirconia.

5. A method as defined in claim 1, wherein the combustible surface is hydrophilic.

6. A method as defined in claim 1, wherein the combustible surface is a plastic film of high surface finish.

7. A method as defined in claim 1, wherein the sharp edges of the meniscus have an edge radius of about 50 nanometers or less.

## Patentansprüche

1. Verfahren zur Herstellung einer Klinge für einen Nassrasierer, umfassend die Schritte:
Bereitstellen eines Substrats, das eine brennbare Oberfläche umfasst;
Erzeugen einer Tinte auf Zirconiumoxidbasis auf der brennbaren Oberfläche, so dass die Tinte das Substrat benetzt und die Ränder des Druckbilds leicht zerfließen, wobei eine Vielzahl von spitzen Menisken entsteht, die als Schneideflächen dienen sollen; und
Brennen der Tinte, so dass die brennbare Oberfläche weggebrannt wird und ein abgerundeter scharfer Rand an der Vielzahl von Menisken gehärtet wird.

2. Verfahren gemäß Anspruch 1, wobei der Schritt des Erzeugens das Aufbringen der Tinte auf Zirconiumoxidbasis durch Siebdruck auf die brennbare Oberfläche umfasst.

3. Verfahren gemäß Anspruch 1, wobei die Tinte auf Zirconiumoxidbasis partiell stabilisiertes Zirconiumoxid umfasst.

4. Verfahren gemäß Anspruch 1, wobei die Tinte auf Zirconiumoxidbasis vollständig stabilisiertes Zirconiumoxid umfasst.

5. Verfahren gemäß Anspruch 1, wobei die brennbare Oberfläche hydrophil ist.

6. Verfahren gemäß Anspruch 1, wobei die brennbare Oberfläche ein Kunststofffilm mit hohem Oberflächenglanz ist.

7. Verfahren gemäß Anspruch 1, wobei die scharfen Ränder des Meniskus einen Kantenradius von etwa 50 Nanometer oder weniger haben.

## Revendications

1. Procédé pour produire une lame pour un rasoir pour rasage humide, comprenant les étapes consistant à :
procurer un substrat avec une surface combustible ;
appliquer une encre à base de zircone sur la surface combustible de manière que l'encre mouille le substrat et les bords de l'impression coulent légèrement pour former une pluralité de ménisques pointus pour servir de surfaces coupantes ; et
cuire l'encre pour brûler la surface combustible et pour durcir un bord tranchant, arrondi sur la pluralité de ménisques.

2. Procédé selon la revendication 1, dans lequel l'étape d'appliquer comprend l'application par sérigraphie de l'encre à base de zircone sur la surface combustible.

3. Procédé selon la revendication 1, dans lequel l'encre à base de zircone comprend du zircone partiellement stabilisé.

4. Procédé selon la revendication 1, dans lequel l'encre à base de zircone comprend du zircone entièrement stabilisé.

5. Procédé selon la revendication 1, dans lequel la surface combustible est hydrophile.

6. Procédé selon la revendication 1, dans lequel la surface combustible est un film en matière plastique avec un fini de surface élevé.

7. Procédé selon la revendication 1, dans lequel les bords tranchants du ménisque ont un rayon de bord d'environ 50 nanomètres ou inférieur.
